

## UNITED STATES PATENT OFFICE

JOHN F. K. McCULLOUGH AND BENJAMIN W. GILCHRIST, OF DETROIT, MICHIGAN,  
ASSIGNORS TO TERNSTEDT MANUFACTURING COMPANY, OF DETROIT, MICHIGAN,  
A CORPORATION OF MICHIGAN

## CHROMIUM PLATING

No Drawing.

Application filed March 26, 1928. Serial No. 264,952.

This discovery relates to chromium plating.

Chromium plating by means of a suitable electrolytic solution and electric current has 5 been proposed years ago. In the early nineties Messrs. Placet and Bonnet disclosed in several foreign and United States patents numerous solutions that were stated to produce good results. These disclosures are very 10 general. Numerous forms of chromium and other metals are stated in one or another of these patents to be capable of use, and the bath capable of being acidulated by almost any kind of an acid. However, the specific 15 disclosures of Placet and Bonnet concerning chromium itself is largely if not wholly confined to chrome sulphates, chrome alums, and chromic acid baths.

Notwithstanding the variety and multiplicity of solutions, baths and acids, which 20 had been stated in the Placet and Bonnet disclosures, practical chromium plating has only in the last few years become active, and this activity is now only in the pioneering stage. 25 Great practical difficulty has been found, largely due to the poor throwing capacity of chromium as compared to nickel and copper, it being found that unless conditions are absolutely right the high spots plate while some 30 of the recesses have little or no coating of chromium. Within the last few years there has been a great deal of investigation and experimental work together with some practical plating, but so far as we are advised, 35 all these baths had been chromic acid ( $\text{CrO}_3$ ) baths. These baths are all founded on the so-called "Sargent" solution, comprising a definite quantity of chromic acid and chromium sulphate. This particular solution has 40 been varied somewhat by the addition of other ingredients, and some stress has been placed in some recent patents upon the proper control of the bath, to wit: the knowledge of exactly how much of a catalyst is present 45 in each bath and the proper maintenance of the relation between the catalyst and the chromic acid by accurately analyzing the bath from time to time, or analyzing the substance added to the bath for traces of impurities in the way of radicals, which alter

the catalyst content of the bath. This literature is here epitomized for the purpose of showing the prevailing practice and the care and nicety which is required in the proper operation of the chromic acid bath, thereby contrasting the wide departure from the prevailing practice which has been accomplished by our bath.

Our bath is founded on the use of chromic chloride and one or more, preferably the three, alkaline metal chlorides,—potassium, sodium and ammonium chloride, with or without other alkaline metal or earth salts such as sodium fluoride, potassium fluoride, ammonium fluoride, or barium, strontium, and calcium fluorides, chlorides, etc. These salts raise the conductivity of the bath and a given voltage will allow the passage of more current, thereby plating more rapidly and consequently effecting economy in plant 70 investment, supervision, etc.

We find it desirable to use a reducing agent for reducing the chromium compounds from higher states of oxidation to lower states of oxidation. We propose to preferably employ soluble chromium or chromium alloy anodes. We find that this reducing agent is desirable in connection with these chromium anodes for the purpose of reducing the hexavalent form of chromium, such as the chromates, to the chromic stage, trivalent. This reduces the chromates into which compounds, among others, the anodes, dissolve to the same stage as the chromic salt with which the bath started, to wit: the chromic chloride. We find that oxalic acid with hydrochloric acid is a suitable reducing agent for reducing the hexavalent chromium to the trivalent chromium.

Hydrochloric acid in small amounts is always found in a bath of this kind, when chromium chloride is dissolved in water. This will serve to combine with the oxalic acid to reduce the hexavalent form of chromium to the trivalent form. This hexavalent form of chromium exists only when soluble chromium anodes are used. After the bath has been going for some time it may be desirable to add more hydrochloric acid in order to react with the oxalic acid to reduce the hex-

avalent form of chromium that accumulates at the anodes. This reaction is as follows:



5 It is therefore desirable to add from time to time amounts of hydrochloric acid and oxalic acid to the bath to reduce the hexavalent chromium in the proportions that are given in the above equation.

10 We are aware that the use of oxalic acid has heretofore been proposed for use in the chromium bath, but it has been proposed for the purpose of acidulating the bath. The 15 purpose of this acidulation is to dissolve the suboxides that are deposited on the cathode. So far as we are aware no acid has been introduced into a chromium bath which has a 20 soluble chromium or chromium alloy anode for the purpose of acting as a reducing agent to reduce the chromates formed by the dissolution of the anode. Certainly no intelligent control and calculation of the bath with 25 this end in view has heretofore been practiced.

We find that an alkaline fluoride such as sodium fluoride is also effective in preventing the precipitation of the basic oxides of chromium on the cathode.

30 The formula that we find very successful is: Chromium chloride ( $\text{CrCl}_3 \cdot 6\text{H}_2\text{O}$ ) 300 grams per liter to saturation (cold), potassium chloride 250 grams per liter to saturation (cold), sodium chloride 250 grams per 35 liter to saturation (cold), ammonium chloride 150 grams per liter to saturation (cold), sodium fluoride 3 to 5 grams per liter (cold), oxalic acid 75 to 100 grams per liter (cold), nitric acid 1%.

40 We find that the nitric acid is desirable in preventing the formation of the chromium oxide, and to act as a depolarizing agent, which facilitates the production of the chromium.

45 We prefer to use chromium chloride in a crystalline form, that is, the hydrated chromic chloride which comes in the form of crystals and has the formula  $\text{CrCl}_3 \cdot 6\text{H}_2\text{O}$ . We use the violet modification of this chromic chloride. It is our understanding that when 50 chromic chloride is dissolved in water three different modifications result, namely: Beta chromic chloride ( $\text{Cr}(\text{H}_2\text{O})_6\text{Cl}_3$ ), violet; alpha chromic chloride

55  $(\text{Cr}(\text{H}_2\text{O})_4\text{Cl}_2)\text{Cl} + 2\text{H}_2\text{O}$ , green in color, and gamma chromic chloride  $(\text{Cr}(\text{H}_2\text{O})_5\text{Cl})\text{Cl} + \text{H}_2\text{O}$ , also green in color. With the violet salt, the solution must 60 be nearly neutral and the temperature must not be too high,—from 80 to 140 degrees Fahrenheit. The acidity is regulated by the addition of caustic soda.

With our bath we use a voltage of from 8 65 to 12, and a current density of from 250 to

1000 amperes per square foot of cathode surface. The higher the temperature at which the bath is operated, the greater the conductivity of the bath and the greater the density of the current. Hence plating can be carried on much faster at the higher ranges of temperature, but the throwing power will not be as good at the higher ranges.

70 We find that the chromium chloride combined with the alkaline metal and earth metal chlorides, in particular, is useful in eliminating the emission of noxious or poisonous gases. This is especially true in avoiding the use of chromium sulphates, including a chromium alum bath. The reaction in such a bath results in the formation of chromic acid. We find it desirable to eschew the joint use of the alkaline chlorides and alkaline sulphates, or any combination of the members of the two groups. These are bound to 75 result in the production of chromic acid. Where chromic acid is formed in a bath of this kind, it reacts with the salts in the bath and free chlorine gas is given off at the anode. This is extremely poisonous. We also find 80 that it is desirable to use a chromium or a soluble chromium alloy anode, even where only the chloride salts are used. Where insoluble anodes are used chlorine gas is released, which does not combine at the anode 85 as is the case where a soluble chromium anode is used.

90 The voltage of 8 to 12, and the amperage of 250 to 1000 is stated at room temperature. It is of course well understood that when the 95 temperature of the bath rises there will be a larger amperage and a smaller voltage. Therefore, when we state our limits of voltage and amperage in the claims, it is understood 100 that this is a relative statement at room temperature, and that this is intended to cover other limits which would be automatically secured by varying the temperature of the bath. It will be apparent that the current 105 density is dependent upon several factors,— the cathode area, the temperature of the bath, the distance between electrodes, voltage, and the alkaline chloride concentration. It is desirable to operate at room temperature, and of course the cathode area depends 110 in a measure upon the work being done, so that the control of the current density largely depends upon the concentration of the conducting salts and the distance between electrodes, and also the regulation of the voltage 115 input. We find that effectual deposition depends largely upon securing substantially the current density we have named.

120 This application is filed as a continuation in part and a substitute for application Serial No. 198,689, filed June 13, 1927.

125 What we claim is:

1. A process for chromium plating which comprises passing an electric current through 130 a bath with a chromium anode and formed

by dissolving in water chromic chloride and one or more of the alkaline metal and earth metal chlorides, and oxalic acid together with nitric acid.

- 5 2. An electro-plating bath in which chromium chloride has been dissolved in water, together with potassium chloride, sodium chloride and ammonium chloride, and substantially the proportions of 300 grams per liter to saturation of the chromium chloride, 250 grams per liter to saturation of the potassium chloride, 250 grams per liter to saturation of the sodium chloride, and 150 grams per liter to saturation of the ammonium chloride, together with 3 to 5 grams per liter of the sodium fluoride.
- 10 3. An electro-plating bath in which chromium chloride has been dissolved in water, together with potassium chloride, sodium chloride and ammonium chloride, and substantially the proportions of 300 grams per liter to saturation of the chromium chloride, 250 grams per liter to saturation of the potassium chloride, 250 grams per liter to saturation of the sodium chloride, and 150 grams per liter to saturation of the ammonium chloride, together with substantially 3 to 5 grams sodium fluoride per liter, 75 to 100 grams oxalic acid, and 1% nitric acid.
- 15 30 In testimony whereof we have affixed our signatures.

JOHN F. K. McCULLOUGH.  
BENJAMIN W. GILCHRIST.

35

40

45

50

55

60

65